

## UNITED STATES PATENT OFFICE

JOHN NAISH GOLDSMITH, OF LONDON, AND THOMAS THORNE BAKER, OF HATCH END, ENGLAND, ASSIGNEES TO SPICERS LIMITED, OF LONDON, ENGLAND, A BRITISH COMPANY

## COLOR PHOTOGRAPHY

No Drawing. Application filed June 20, 1930, Serial No. 462,697, and in Great Britain July 30, 1929.

This invention consists in improvements in or relating to color photography, and particularly to the production of photographic films which carry a reseau or multicolor screen as well as a sensitized emulsion. Films of this type can be used for taking photographs, or for reproduction of photographs or for cinematograph films in natural colors.

10 By means of the process described in pending application Serial No. 345604 L. Dufay, filed 8th March, 1929, successful results have been achieved in applying the multicolor screen to a film made of cellulose acetate composition.

The object of the present invention is to enable the multicolor screen to be successfully applied to cinematographic films of various kinds, including films made from celluloid, from cellulose nitrate, from viscose and the like.

Taking the simple case where a film is to receive (1) A dye of one color, say green; (2) A series of lines of a resist (such, for example as fatty ink); (3) Treatment with a bleaching or color-discharging liquid; (4) A dye with another color in the spaces thus bleached; a further object of this invention is to ensure that the dyed zones of the film shall be such that the discharge of color therefrom, and the application of another color, shall be readily accomplished without "creeping" under the resist lines, and without masking of one color by another so that, in fact, the separate color elements are clearly distinct and have their proper color values. Another object is to ensure uniformity of the color value or intensity from side to side of each line of color.

40 According to this invention, it has been found that with any given "base" (i. e. with a supporting film which may be celluloid, cellulose, cellulose nitrate or other ester or ether of cellulose) and where a special surface layer is to be used which is to receive the dyes, and from which dye can be discharged, it is possible to isolate the surface layer from the base by an intermediate layer or septum.

45 According to the invention a film of celluloid, viscose, cellulose nitrate or other ester

or ether of cellulose is prepared for color photography by coating the basic film with a layer of isolating material, then with a surface layer of a material amenable to dyes and to discharging agents, and applying to 55 the film thus prepared a multicolor screen.

According to the feature of the invention the surface layer which is to receive the dyes consists of cellulose nitrate, collodion, cellulose prepared from viscose or other cellulose solution, or other similar material which will readily receive and permit of the subsequent discharge of dyes.

The isolating layer differs from the other two layers either in chemical composition or 65 in physical properties or in both. The function of the isolating layer is to locate substantially or completely the dyeing and discharging operations in the surface layer, or in other words to inhibit the penetration of 70 dyeing agents or discharging agents into the film base. The isolating layer may be produced from a solution of cellulose acetate with or without added agents such as plasticizing agents; again, the isolating layer 75 may be a condensation product of formaldehyde and phenol or thiourea, or it may be a varnish or coating of other synthetic resin.

The following is a description by way of example of one method of carrying this invention into effect in making a cinematograph film in natural colors with a base of celluloid.

The celluloid film is passed round a roller which dips into a bath containing a 14-15% 85 solution of cellulose acetate in acetone with sufficient plasticizers (i. e. about 5-6%) to prevent the dry film from curling. By this means a coating of cellulose acetate whose thickness is of the order of from 4-8 $\mu$  may 90 be applied to the surface of the celluloid film. If the 15% solution of cellulose acetate is found to be too viscous, its viscosity may be reduced by addition of further quantities of solvent. The cellulose acetate solution 95 may, if desired be prepared by dissolving cellulose acetate film, such for example as scrap commercial film, in acetone. In this manner the desired quantity of plasticizers will be incorporated in the solution. 100

Further there may be added to the solution of cellulose acetate higher boiling solvents, such as cyclohexanone.

When this acetate film is dry the film is passed again through a film-coating machine and there is applied thereto a fine coating (surface layer) of collodion. Conveniently, this surface layer contains one of the dyes, for example a green dye such as malachite green.

Now proceeds the process of applying the reseau or multicolor screen.

The film (the surface layer of which is dyed uniformly green all over) is then led through a printing machine by means of which extremely fine parallel lines of a resist (such, for example, as a greasy ink) are printed upon it. The printing may be effected by means of a small engraved steel roller having (in one case) 15 lines and 15 intervening grooves per millimetre. The film at this stage exhibits 15 clear green lines and 15 opaque greasy lines (green underneath) per millimetre, both kinds of lines being of about the same width. After an interval to let the ink dry the film is led in succession (a) over a bath which bleaches and dissolves out the green dye from only the clear spaces, leaving unattacked the green lines protected by the ink; (b) over an inking roller which applies a red dye to the spaces between the ink lines, after which the film is thoroughly washed with water to remove excess of dye; (c) through a solvent cleansing bath of benzene to remove the ink lines, leaving exposed the clear green lines.

The film is again led (when dry) through the printing machine which produces parallel lines of a resist (such as greasy ink) as before, but this time at right angles to those formerly made. After an interval for the ink to dry the film is led in succession (a) over a bath which bleaches and dissolves out the red and green dye from only the clear spaces between the greasy lines, (b) over an inking roller which applies a violet dye which dyes the interline spaces, and (c) through a solvent cleansing bath of benzene. The film is then dried, is coated with a suitable sub-stratum and is thereafter coated with a layer of sensitized emulsion (a panchromatic emulsion).

We claim:—

1. A method of preparing a film comprising a cellulose derivative for color photography which comprises coating the film base first with an isolating material to inhibit the penetration of solutions of dyes and discharging agents into the film base, then with a surface layer of a material amenable to dyes and to discharging agents, and finally applying to the said surface layer of the film thus prepared a multi-color screen.

2. A method of preparing a film comprising a cellulose ester for color photography

which comprises coating the film base first with an isolating material to inhibit the penetration of solutions of dyes and discharging agents into the film base, then with a surface layer of a material amenable to dyes and to discharging agents, and finally applying to the said surface layer of the film thus prepared a multi-color screen. 70

3. A method of preparing a film comprising celluloid for color photography which comprises coating the film base first with an isolating material to inhibit the penetration of solutions of dyes and discharging agents into the film base, then with a surface layer of a material amenable to dyes and to discharging agents, and finally applying to the said surface layer of the film thus prepared a multi-color screen. 75

4. A method of preparing a film comprising a cellulose derivative for color photography which comprises coating the film base first with an isolating material to inhibit the penetration of solutions of dyes and discharging agents into the film base, then with a surface layer of a solution of a cellulose derivative which is amenable to dyes and to discharging agents, and finally applying to the said surface layer of the film thus prepared a multi-color screen. 80

5. A method of preparing a film comprising a cellulose derivative for color photography which comprises coating the film base first with an isolating material to inhibit the penetration of solutions of dyes and discharging agents into the film base, then with a surface layer of collodion, and finally applying to the said surface layer of the film thus prepared a multi-color screen. 90

6. A method of preparing a film comprising a cellulose derivative for color photography which comprises coating the film base first with a solution of cellulose acetate, then with a surface layer of a material amenable to dyes and to discharging agents, and finally applying to the said surface layer of the film thus prepared a multi-color screen. 105

7. A method of preparing a film comprising a cellulose derivative for color photography which comprises coating the film base first with a solution of cellulose acetate containing plasticizers, then with a surface layer of a material amenable to dyes and to discharging agents, and finally applying to the said surface layer of the film thus prepared a multi-color screen. 115

8. A method of preparing a celluloid film for color photography, which comprises first applying to the film a solution of cellulose acetate in acetone containing plasticizers so as to obtain an isolating coating of cellulose acetate of thickness from 4-8 $\mu$ , then applying a surface layer of collodion, and finally applying to the said surface layer of the film thus prepared a multi-color screen. 125

9. A method of preparing a celluloid film 130

for color photography, which comprises first applying to the film a 15% solution of cellulose acetate in acetone containing plasticizers so as to obtain an isolating coating of cellulose acetate of thickness from 4-8 $\mu$ , then applying a surface layer of collodion, and finally applying to the said surface layer of the film thus prepared a multi-color screen.

10. A method of preparing a celluloid film for color photography, which comprises first applying to the film a 15% solution of cellulose acetate in acetone containing 5-6% of plasticizers, then applying a surface layer of collodion, and finally applying to the said surface layer of the film thus prepared a multi-color screen.

11. A method of preparing a film comprising a cellulose derivative for color photography which comprises coating the film base first with an isolating material to inhibit the penetration of solutions of dyes and discharging agents into the film base, then applying a surface layer of a material amenable to dyes and to discharging agents, and finally applying to the said surface layer thus prepared a multi-color screen by a process including the use of dyes, resists and dye-discharging agents.

12. A method of preparing a film comprising a cellulose derivative for color photography which comprises coating the film base first with an isolating material to inhibit the penetration of solutions of dyes and discharging agents into the film base, then applying a surface layer of a solution of a cellulose derivative which is amenable to dyes and to discharging agents, and finally applying to the said surface layer thus prepared a multi-color screen by a process including the use of dyes, resists and dye-discharging agents.

13. A method of preparing a film comprising a cellulose derivative for color photography which comprises coating the film base first with a solution of cellulose acetate containing plasticizers, then applying a surface layer of a material amenable to dyes and to discharging agents, and finally applying to the said surface layer thus prepared a multi-color screen by a process including the use of dyes, resists and dye-discharging agents.

14. A film adapted for use in color photography comprising a cellulose derivative base, a layer of isolating material capable of inhibiting the penetration of dyes and discharging agents into the cellulose derivative base, a surface layer on said isolating layer amenable to dyes and discharging agents carrying a multi-color screen in which the separate color elements are clearly distinct.

15. A film adapted for use in color photography comprising a celluloid base, an isolating coating of cellulose acetate containing

plasticizers, a surface layer on said isolating layer amenable to dyes and discharging agents carrying a multi-color screen in which the separate color elements are clearly distinct.

16. A film adapted for use in color photography comprising a celluloid base, an isolating coating 4-8 $\mu$  thick of cellulose acetate containing plasticizers, and a surface layer on said isolating layer amenable to dyes and discharging agents and carrying a multi-color screen in which the separate color elements are clearly distinct.

17. A film adapted for use in color photography comprising a cellulose derivative base, a layer of isolating material capable of inhibiting the penetration of dyes and discharging agents into the cellulose derivative base, and a surface layer of collodion on said isolating layer carrying a multi-color screen in which the separate color elements are clearly distinct.

18. A film adapted for use in color photography comprising a celluloid base, an isolating coating of cellulose acetate containing plasticizers, and a surface layer of collodion on said isolating layer amenable to dyes and discharging agents and carrying a multi-color screen in which the separate color elements are clearly distinct.

19. A film adapted for use in color photography comprising a celluloid base, an isolating layer of thickness from 4-8 $\mu$  of cellulose acetate containing 5-6% of plasticizers and a surface layer of collodion on said isolating layer carrying a multi-color screen in which the separate color elements are clearly distinct.

In testimony whereof we have signed our names to this specification.

JOHN NAISH GOLDSMITH.  
THOMAS THORNE BAKER.

70

75

80

85

90

95

100

105

110

115

120

125

130